

Patented June 30, 1925.

1,543,921

## UNITED STATES PATENT OFFICE.

BERT MACE HUFF, OF DETROIT, MICHIGAN, ASSIGNOR OF ONE-THIRD TO HAROLD A. ARNOLD, OF DETROIT, MICHIGAN, AND ONE-THIRD TO MAURICE E. FITZGERALD, OF PONTIAC, MICHIGAN.

### METALLIC ALLOY..

No Drawing.

Application filed January 28, 1924. Serial No. 639,149.

To all whom it may concern:

Be it known that I, BERT MACE HUFF, a citizen of the United States of America, residing at Detroit, in the county of Wayne 5 and State of Michigan, have invented certain new and useful Improvements in Metallic Alloys, of which the following is a specification.

The invention relates to metallic alloys 10 and more particularly to a non-ferrous type suitable for the manufacture of cutting tools. The object of the invention is to produce an alloy having great hardness and toughness, one that will not be susceptible 15 to ready oxidation and that may be welded and will have other desirable properties for use as a cutting tool.

The principal ingredients of my new alloy are cobalt, chromium and tungsten and, 20 while these elements have heretofore been used in the manufacture of non-ferrous cutting alloys, I have found that by properly proportioning the percentages of these elements and adding thereto certain amounts 25 of other elements it is possible to obtain a cutting alloy having qualities superior to any of the commercial alloys of this general nature. Amongst the elements which may be added to cobalt, chromium and tungsten to produce a better alloy are manganese and silicon and these are preferably present to the amount of about one 30 percent each.

As a typical example of my improved 35 alloy the following complete analysis is submitted:

|             | Per cent. |
|-------------|-----------|
| Cobalt      | 45.72     |
| Chromium    | 30.96     |
| 40 Tungsten | 12.82     |
| Iron        | 4.14      |
| Carbon      | 2.37      |
| Manganese   | 1.03      |
| Silicon     | 0.98      |
| 45 Nickel   | 0.97      |
| Calcium     | 0.34      |
| Magnesium   | 0.08      |
| Phosphorus  | 0.04      |
| 50 Total    | 99.45     |

tively pure materials, the chromium and tungsten being ninety-five percent (95%) 55 pure and the cobalt ninety percent (90%) pure. It is also preferable to introduce the manganese and silicon by adding to the above metals the proper proportions of manganese and silicon, each approximately 60 ninety percent (90%) pure. It is also desirable to introduce a small amount of iron into the mixture, preferably in the form of malleable or Norway iron. The materials are mixed in the desired proportions 65 and melted, preferably in an electric arc furnace under a temperature of approximately 2800 degrees Fahrenheit, and when thoroughly molten the alloy is cast into chills. The resulting product is found to 70 be exceedingly hard, tough, non-magnetic, and weldable, and cannot be machined by ordinary methods.

While the above analysis has been given 75 to show a typical alloy embodying my invention, I wish it understood that I do not restrict myself to the exact percentages mentioned therein for it is obvious that some of the elements of the analysis are present only as impurities and might be eliminated by more careful selection of the materials used in the manufacture. However, I have found that extremely good results are obtained by using materials of the purity indicated.

As illustrative of the range of the different elements in the alloy the following figures are submitted as representing the limits of my preferred composition, although I wish it understood that I do not 90 regard myself as being necessarily limited by these percentages except as denoted in the appended claims:

|           | Per cent. | Minimum | Maximum |
|-----------|-----------|---------|---------|
| Cobalt    | 40.00     | 50.00   | 95      |
| Chromium  | 25.00     | 35.00   |         |
| Tungsten  | 5.00      | 15.00   |         |
| Iron      |           | 5.00    |         |
| Carbon    | 1.00      | 4.00    |         |
| Manganese | 1.00      | 1.50    |         |
| Silicon   | 1.00      | 5.00    | 100     |

The carbon in the alloy may be introduced combined with the other materials, such, for instance, as the malleable iron and 105 it is sometimes also introduced by absorp-

In the manufacture of an alloy of the above analysis, it is preferable to use rela-

tion from the crucible or the carbon electrodes of the arc furnace.

What I claim as my invention is:—

1. A metallic alloy containing as the 5 principal ingredient substantial amounts of cobalt, chromium and tungsten totaling not less than 70% together with relatively small amounts of manganese and silicon, the cobalt not exceeding 50%, the chromium not 10 exceeding 35% and the tungsten not exceeding 15%.

2. A metallic alloy containing cobalt from 15% to 50%, chromium from 25% to 35%, tungsten from 5% to 15% together with small amounts of manganese and silicon.

3. A metallic alloy containing cobalt from 40% to 50%, chromium from 25% to 35%, tungsten from 5% to 15%, carbon from 1% to 4%, manganese from 1% to 1 $\frac{1}{2}$ %, and 20 silicon from 1% to 5%.

4. A metallic alloy containing cobalt, approximately forty-six percent (46%), chromium, approximately thirty-one percent (31%), tungsten, approximately thirteen 25 percent (13%), together with small amounts of iron, manganese and silicon.

5. A metallic alloy containing cobalt, approximately forty-six percent (46%), chromium approximately thirty-one percent 30 (31%), tungsten, approximately thirteen

percent (13%), together with small amounts of iron, manganese, silicon and carbon.

6. A metallic alloy containing cobalt, approximately forty-six percent (46%), chromium, approximately thirty-one percent (31%), tungsten, approximately thirteen percent (13%), iron, approximately four percent (4%), carbon, approximately two and five-tenths percent (2.5%), manganese, approximately one percent (1%), and silicon, approximately one percent (1%).

7. A metallic alloy consisting of the ingredients in the proportions substantially as follows:

|            | Per cent. |
|------------|-----------|
| Cobalt     | 45.72     |
| Chromium   | 30.96     |
| Tungsten   | 12.82     |
| Iron       | 4.14      |
| Carbon     | 2.37      |
| Manganese  | 1.03      |
| Silicon    | 0.98      |
| Nickel     | 0.97      |
| Calcium    | 0.34      |
| Magnesium  | 0.08      |
| Phosphorus | 0.04      |

In testimony whereof I affix my signature.

BERT MACE HUFF.